

## UNITED STATES PATENT OFFICE.

PETER OSTENDORF, OF BERNDORF, AUSTRIA.

## COPPER AND ZINC ALLOY.

No Drawing.

Application filed October 4, 1922. Serial No. 592,411.

*To all whom it may concern:*

Be it known that I, PETER OSTENDORF, a Prussian subject, residing at Berndorf, Lower Austria, have invented new and useful Improvements in and Relating to Copper and Zinc Alloys, of which the following is a specification.

Copper and zinc alloys containing more than 40% of zinc which have been improved 10 by the addition of nickel and manganese, are known.

These known alloys however, cannot be worked when cold as they are far too brittle. On the other hand, copper and zinc alloys 15 containing less than 40% of zinc cannot be worked when hot.

For many purposes it is of the greatest importance to obtain an alloy which can be easily worked both cold as well as hot, as 20 many articles made from such alloys have to be worked both whilst hot as well as cold in order to give them the particular form required.

It has been found that copper and zinc 25 alloys, easily worked both cold and hot, can be obtained if a preponderating percentage of copper and zinc is alloyed with nickel and manganese, in the presence of a certain proportion of aluminium.

In practice it has been found that an addition of 2% of aluminium produces an alloy satisfactory in every respect, and capable of being worked when hot or cold. The addition of aluminium however, must 35 not exceed 3%, as otherwise the alloy will again become brittle and unworkable when cold.

It is important that the quantity of zinc in alloys of the kind referred to should under 40 no circumstances exceed 40% and should be greater than 25%.

In addition to the constituents already referred to, the improved alloy may also have admixtures of manganese and iron added 45 to it.

The invention consists in mixing together copper, nickel, manganese, iron, 25 to 40% of zinc and  $\frac{1}{2}$  to 3% of aluminium, the copper, nickel, manganese and iron being melted 50 together, the zinc added to the molten

mixture and finally after some minutes introducing the aluminium.

Such an alloy may consist, for instance of 40-55 parts of copper, 3-15 parts of nickel, 1-3 parts of manganese, 1-2 parts of iron, 55 0.5-3 parts of aluminium and less than 40 parts of zinc. A particularly good alloy consists of 48 parts of copper, 10 parts of nickel, 3 parts of manganese, 2 parts of iron, 2 parts of aluminium and 35 parts of 60 zinc.

When compounding the alloy, a charge consisting of the required amount of the copper, nickel, manganese, and iron is first melted, the zinc is then added and after 65 some minutes the aluminium is introduced. After thorough mixing the alloy may be cast in bars, or in any shape desired.

In the improved alloy, nickel, manganese and iron are the principal factors of 70 strength, while the limited quantity of zinc, and the percentage of aluminium kept within the correct limits, cause the alloy to be workable both whilst cold or hot; it has a very fine grain; is very dense and very 75 resistant to chemical action compared with known copper and zinc alloys and is therefore capable of being used advantageously for articles requiring the characteristics recited.

I claim:

1. An improved alloy consisting of 40 to 55 parts by weight of copper, 3 to 15 parts by weight of nickel, 1 to 3 parts by weight of manganese, 1 to 2 parts by weight of iron,  $\frac{1}{2}$  to 3 parts by weight of aluminium and 25 to 40 parts by weight of zinc.

2. An improved alloy consisting of 48 parts by weight of copper, 10 parts by weight of nickel, 3 parts by weight of manganese, 2 parts by weight of iron, 2 parts by weight of aluminium and 35 parts by weight of zinc.

In testimony whereof I have signed this specification in the presence of two witnesses.

P. OSTENDORF.

Witnesses:

CARL WIEDENBERG,  
JOHANN KUHN.